

March 12, 1935.

N. C. RENDLEMAN

1,994,287

METHOD OF MAKING PLOWSHARES

Filed June 20, 1933

2 Sheets-Sheet 1



March 12, 1935.

N. C. RENDLEMAN

1,994,287

METHOD OF MAKING PLOWSHARES

Filed June 20, 1933

2 Sheets-Sheet 2



INVENTOR  
Norman C. Rendleman  
by his attorney

Byrnes, Stebbins, Parmelee & Blenko

## UNITED STATES PATENT OFFICE

1,994,287

## METHOD OF MAKING PLOWSHARES

Norman C. Rendleman, Pittsburgh, Pa., assignor  
to Jones & Laughlin Steel Corporation, Pitts-  
burgh, Pa., a corporation of Pennsylvania

Application June 20, 1933, Serial No. 676,624

10 Claims. (Cl. 29—14)

My invention relates to a plow share or point and a method of manufacturing such article.

The manufacture of plow shares as carried on heretofore by welding the landside portion 5 onto the blade portion, and trimming and forging the welded assembly, has been expensive and wasteful of stock. Because of the irregular shape of the article, the scrap loss has often run as high as 40 percent.

10 In accordance with my invention, I avoid the high scrap loss characterizing previous methods of manufacturing plow shares. I take flat bar stock and subject it to die rolling to form certain portions of the finished share, specifically 15 the blade and a part of the landside. The die rolled bar thus constitutes a string of partial or blade and landside blanks for the manufacture of shares. In the die rolling, raised ribs are formed extending transversely of the bar 20 and at an angle to the length thereof. I subject a second piece of bar stock to a die rolling operation in which substantially similar ribs are formed. The second die rolled bar or string of blanks is then cut into triangular pieces to 25 form the toes and heels of the shares. These pieces are flash welded to the blanks formed by the first die rolling operation so that the ribs of the triangular pieces form a continuation of the ribs of the partial blanks. The completed 30 blanks are then sheared and subjected to bending and forging operations to impart thereto the desired final shape.

For a complete understanding of the invention, reference is made to the accompanying 35 drawings illustrating a preferred practice. In the drawings:

Figure 1 is a plan view of a string of blade and landside blanks formed by die rolling a length of bar stock;

40 Figure 2 is a side elevation of the string shown in Figure 1;

Figure 3 is a view largely diagrammatic illustrating the die rolling operation which produces the string of blanks shown in Figures 45 1 and 2;

Figure 4 is a view similar to Figure 1 showing two blade and landside blanks of equal length sheared from the string shown in Figures 1 and 2;

50 Figure 5 is a view similar to Figure 4 showing two partial blanks of different lengths sheared from the same string;

Figure 6 is a view similar to Figure 1 showing 55 the string of toe and heel blanks formed by a

die rolling operation in the same manner as the string of Figures 1 and 2;

Figure 7 is a side elevation of the string of Figure 6;

Figure 8 is a view similar to Figure 4 illustrating the manner of positioning the toe and heel blanks adjacent the partial blanks preparatory to welding them together;

Figure 9 is a view similar to Figure 8 showing the parts assembled within a jig for welding; 10

Figure 10 is a sectional view substantially along the line X—X of Figure 9 illustrating diagrammatically the welding of the parts;

Figure 11 is a plan view of two complete 15 blanks for shearing and trimming;

Figure 12 is a similar view of a complete blank after shearing and trimming;

Figure 13 is an edge view of the blank after it has been subjected to a preliminary bending operation;

Figure 14 is a similar view showing the blank after it has been subjected to a forging operation;

Figure 15 is a sectional view along the line 20 XV—XV of Figure 14; and

Figure 16 is a perspective view of the finished share showing the shaped blade and heel and an inserted point of hard steel welded in place.

Referring now in detail to the drawings, I take a piece of flat bar stock 10 of suitable dimensions and subject it to die rolling between rolls 11 and 12 to produce a string 13 of partial blanks 14. The die roll 11 is suitably grooved at 15 to form ribs 16 extending transversely of the blanks 14 in pairs at an angle to the length 30 thereof. An open pass is used and the blanks are slightly widened, as shown at 17.

As shown in Figure 1, the ribs 16 are formed in pairs along the length of the string 13. The string may be sheared into pieces by cutting between the pairs of ribs to form sets of two partial blanks secured together in reversed, opposed relation as shown in Figures 4 and 5. Each end of each piece includes a blade-forming portion 18 and at least a part of a landside 35 19. The ribs 16 are formed at the junction of the portions 18 and 19.

By shearing the string along the dotted lines aa in Figure 1, it will be apparent that two connected partial blanks of substantially the same 50 length of blade will be formed, as shown in Figure 4, whereas by shearing the string along the dotted lines bb, two connected partial blanks having different lengths of blade will be formed, as shown in Figure 5. The grooves 15 in the 55

roll 11 will be such as to provide also a suitable amount of excess material between adjacent sets of blanks to permit some tolerance in the shearing of the string without introducing an inordinate amount of waste.

In the manner already described for the formation of the partial blanks 14, I die roll flat bar stock to produce a string of toe and heel blanks illustrated at 20. The toe and heel blanks are characterized by ribs 21 extending thereacross in the same manner as the ribs 16 are positioned on the blanks 14, and by slight spreadings 22 on opposite sides of the ribs 21. I shear the string 20 into blanks along the dotted lines 23 and 24. It will be apparent that this operation produces a plurality of identical blanks of substantially triangular outline, each blank having a raised rib extending substantially from one vertex of the triangle to the midpoint of the opposite side. The separate toe and heel blanks are illustrated at 25 in Figure 8 where they are shown disposed in proper relation to the blanks 14 prior to welding thereto. Each of the blanks 25 has a portion 26 adapted to cooperate with the portion 19 of the blanks 14 to form the heel of a finished share. The remaining portion 27 of the blanks 25 cooperates with the blade-forming portion 18 of the blanks 14 to form the toe of the shares.

When the partial blanks 14 and the toe and heel blanks 25 have been disposed as shown in Figure 8, they are brought together and placed within a jig, as shown in Figure 9, comprising movable plates 28 and 29 having upstanding lugs 30 thereon. It will be observed in Figures 8 and 9 that the ribs 21 of the toe and heel blanks are in alignment with the ribs 16 of the blade and landside blanks 14. The jig plates 28 and 29 may be actuated and controlled in any suitable manner to press the blanks 25 toward the partial blanks 14. While the parts are in such relation, I supply electric current to the joints between the toe and heel blanks and the partial blanks to effect welding thereof, preferably by some such means as shown in Figure 10, comprising a pair of welding electrodes 31, each electrode having an insulated portion adapted to contact with and supply current to the associated blanks on opposite sides of the joint therebetween.

The passage of electric current across the joints between blanks heats the edge portion of the latter in the known manner and simultaneous operation of the jig plates 28 and 29 will force the heated edges together to effect a satisfactory weld. In the welding operation, the overfilled portions 17 and 22 of the blanks provide the necessary excess metal which is forced out of the welded seam as flash. This may be removed in any convenient manner. The result of the welding operation, as shown in Figure 11, is a pair of complete share blanks 32 and 33. The two blanks of each pair are obviously arranged in opposed, reversed relation.

When the completed pair of blanks, shown in Figure 11, are sheared apart along the line 34 extending substantially from the outer vertex of one of the blanks 25 to a similar point of the other toe and heel blank, two identical share blanks are formed which, after a suitable trimming operation along the lines 35, have the appearance shown in Figure 12. The completed blank has a blade 36 which is substantially identical with the blade-forming portion 18 of the partial blank 14. The completed blank also has

a landside 37 formed by the portion 19 of the blank 14. The portion 26 of the blank 25 forms the heel of the landside. The toe 38 of the completed blank is formed by the remainder of the blank 25 which is left after the removal of the heel-forming portion 26 thereof. The blade 36, the landside 37 and the toe 38 of the finished blank, shown in Figure 12, are disposed substantially in the same plane. The finished blank must, obviously, be subjected to certain forming operations to bring the several portions thereof into proper relation.

Figure 13 illustrates the condition of the blank after the landside 37 has been bent substantially at right angles to the blade 36. When the landside and blade have thus been bent, the blank is subjected to a forging operation which imparts a slight curvature to the blade 36, bends the landside 37 slightly beyond its initial right angular position, and brings the other parts of the article into the shape and relation shown in Figure 14. A hard steel piece 40 is welded onto the toe. The share is then ready for such machining operations as are necessary to adapt it for assembly with the remaining parts of a plow.

It will be apparent from the foregoing description that the invention provides a highly efficient method of making plow shares or points. The amount of scrap produced in the practice of the method is obviously quite small and, the various parts making up the completed share may readily be produced very cheaply and rapidly by die rolling which is already well known. The cost of shares made in accordance with my invention will obviously be much less than those produced by the old forging process, not only because of the reduction in the amount of scrap but also because of the rapid rate and low cost at which the necessary components of the finished share may be turned out.

Although I have illustrated and described herein but one preferred practice of the invention, it will be apparent that numerous changes therein may be made without departing from the spirit of the invention or the scope of the appended claims.

I claim:

1. In a method of making plow shares, the steps including die rolling a leader to form a string of partial blanks, each having portions adapted to constitute the blades and landsides of a pair of completed shares, and a pair of parallel ribs on one surface extending at an angle to the length of the string, constituting the junctions of said portions, die rolling a second leader to form a string of toe and heel blanks, said string having uniformly spaced parallel ribs extending at an angle to the length of the string, shearing the second string into similar triangular toe and heel blanks, the ribs of each extending substantially from one vertex to the midpoint of the opposite side, welding the toe and heel blanks to opposite sides of the partial blanks with the ribs of the former in line with the ribs of the latter, shearing the partial blanks substantially along a line connecting the outer ends of the ribs of the point blanks to form two complete share blanks, trimming each complete blank, bending the landside portion of each blank at an angle to the blade portion and forging the blanks.

2. In a method of making plow shares, the steps including die rolling a leader to form a string of partial blanks, each having portions adapted to constitute the blades and portions of the land-

sides of a pair of completed shares, and a pair of parallel ribs on one surface extending at an angle to the length of the string, die rolling a second leader to form a string of toe and heel blanks having uniformly spaced parallel ribs extending at an angle to the length of the string, shearing the second string into similar triangular toe and heel blanks, welding the toe and heel blanks to opposite sides of the partial blanks with the ribs of the former in line with the ribs of the latter to form a pair of complete blanks, shearing the welded blanks to form two complete share blanks, bending the landside portion of each blank at an angle to the blade portion and forging the blanks.

3. In a method of making plow shares, the steps including die rolling a leader to form a string of partial blanks, each having portions adapted to constitute the blades and portions of landsides of a pair of completed shares, shearing the partial blanks from the string, die rolling a second leader to form a string of toe and heel blanks, shearing the second string into similar triangular point blanks, welding the toe and heel blanks to opposite sides of the partial blanks, shearing the welded blanks to form two complete share blanks, and forging the blanks to shape.

4. In a method of making plow shares, the steps including die rolling a leader to form a string of pairs of blanks, each blank having portions adapted to constitute the blade and a portion of the landside of a share, shearing the pairs from the string, die rolling a second leader to form a string of toe and heel blanks, shearing the second string to form individual toe and heel blanks, welding the toe and heel blanks to opposite sides of the pairs of blanks, shearing the pairs of blanks to form two complete share blanks from each and forging the blanks to shape.

5. In a method of making plow shares, the steps including die rolling a bar to form a string of partial share blanks each having blade and landside-forming portions, shearing pairs of blanks from the string, die rolling a second bar to form a string of toe and heel blanks, shearing

the toe and heel blanks apart and welding them to opposite sides of the pairs of blanks from the first-mentioned string to form complete share blanks, shearing the pairs of blanks apart and forging the blanks to shape.

6. In a method of making plow shares having a toe, a blade and a landside with a heel, the steps including die rolling a leader to form blanks having portions adapted to constitute the blade and a part of a landside of a finished share, die rolling a second leader to form blanks adapted to constitute the toe and heel of a finished share, shearing the toe and heel blanks apart and welding them on the first-mentioned blanks, shearing the first-mentioned blanks apart, and forging the completed blanks to shape.

7. In a method of making plow shares having a toe, blade, and landside, the steps of die rolling bar stock to form blanks, including in an integral piece certain of said portions, shearing the blanks into combinations of two each, die rolling a second piece of bar stock to form blanks containing other parts of said portions, shearing the last-mentioned blanks apart and welding them to opposite sides of said combinations, to form pairs of complete blanks, shearing the pairs of blanks apart and forging the blanks so formed.

8. The method of claim 6 characterized by shearing the first-mentioned blanks into pairs before welding the toe and heel blanks thereto, and finally shearing the pairs of complete blanks on a line through the first-mentioned blanks and the toe and heel blanks welded thereto.

9. The method of claim 6 characterized by shearing the blade blanks into pairs and welding a toe and heel blank onto both sides of the pair of blade blanks.

10. The method of claim 6 characterized by shearing the blade blanks into pairs and welding a toe and heel blank onto both sides of the pair of blade blanks, and separating the blanks of each pair so as to leave a portion of both toe and heel blanks.

NORMAN C. RENDLEMAN.